

1,342,801.

C. L. GEBAUER.  
PROCESS OF PRODUCING METAL BODIES.  
APPLICATION FILED MAY 17, 1917.

Patented June 8, 1920.



Fig. 1



Fig. 2.

Inventor,  
Charles L. Gebauer  
By Will Smith Beck West.  
A. T. G.

# UNITED STATES PATENT OFFICE.

CHARLES L. GEBAUER, OF CLEVELAND, OHIO.

## PROCESS OF PRODUCING METAL BODIES.

1,342,801.

Specification of Letters Patent.

Patented June 8, 1920.

Application filed May 17, 1917. Serial No. 169,176.

*To all whom it may concern:*

Be it known that I, CHARLES L. GEBAUER, a citizen of the United States, residing at Cleveland, in the county of Cuyahoga and 5 State of Ohio, have invented a certain new and useful Improvement in Processes of Producing Metal Bodies, of which the following is a full, clear, and exact description, reference being had to the accompanying 10 drawings.

This invention relates to a new process of producing metal bodies, the metal bodies in question being themselves of peculiar construction and valuable properties. In my 15 copending application filed April 12, 1916, Serial No. 90,585, I have described and claimed an alloy and process of producing same wherein a metal of high fusing point and a metal of lower fusing point being first 20 reduced to finely pulverized form are mixed intimately together, pressed into form and finally heated to such a temperature as to melt the more fusible ingredient and cause it to embrace the less fusible ingredient. Further 25 experiments have disclosed the fact that it is not necessary in all cases to mix two metals together, but that if the less fusible ingredient be reduced to pulverized form and very forcibly compacted, the more fusible ingre- 30 dient can be introduced or sweated into the mass from the outside, at least sufficiently for practical purposes in many applications. This procedure is especially convenient prac- 35 tically from the fact that most of the high fusing point metals can be obtained rather easily in pulverized form whereas it is frequently very difficult to secure the more fusible metals in this condition.

While I do not limit myself to the use 40 of any particular metal or of any combina- 45 tion or combinations of metals, I prefer to use and for practical purposes have used a combination of tungsten and platinum more frequently than any others, as for example in the construction of parts for electrical instruments such as spark points or arcing terminals. In the performance of my said invention, assuming the above named mate- 50 rials to be employed, the tungsten is utilized in the finely divided crystalline form just as it is derived from the reduction of tungstic 55 oxid by hydrogen. This finely granular ma- terial is first compacted under great pressure, as by a hydraulic or other press, into the exact shapes and sizes required. The articles are then placed in a suitable heating device

such as an electric furnace, in close surface contact with sheets or plates or layers of the other substance. Thus in the case of spark points, a disk of platinum foil of the appropriate size is laid on top of each member, while for rods or bars the foil is wrapped around the same, or for irregular shapes a layer of finely divided platinum (or other metallic substance) can be sprinkled thereon. 60 The furnace then being heated to the regular temperature, the more fusible metal is first melted and then absorbed by the less fusible article. A reducing or neutral atmosphere is maintained in the furnace during this op- 70 eration so as to prevent any such oxidation of the metal as would impede close surface contact. The rate and amount of absorption can be regulated by the porosity of the articles, this being dependent upon the coarse- 75 ness of the pulverization and the pressure employed in compacting. In the case of tungsten, molybdenum, and the like metals, which are reduced by hydrogen, the crystal size can be modified by proper regulation of 80 temperature during the reduction as is well known. A sufficiently close compacting must be given in all cases to enable the articles to withstand reasonable handling prior to the sweating or impregnating operation. 85

In addition to the convenience gained by the ability to use each metal in the form in which it is most cheaply obtained com- 90 mercially, there is the consideration that less of the more fusible substance is employed than when the two substances are mixed uniformly together, and this substance is located in large proportion at the place where it is most useful, namely adjacent to the surface of the resulting article. 95

A great many combinations of metals can be employed, though preferably they should be so chosen as not to be mutually soluble under the conditions described. I can see that my invention will be most useful in 100 cases where tungsten, molybdenum, and the like constitute the more refractory element, and platinum, silver or gold the more fusible element, but I do not confine myself thereto. Ordinarily the more fusible metal constitutes 105 from 3 to 10 percent. of the weight of the less fusible metal but these proportions are also susceptible to variation according to the par- ticular use in view.

In the accompanying drawings, Figure 1 110 is an elevational view of a contact point em- bodying my invention, and Fig. 2 is a view

of a portion of the working surface thereof on an exaggerated scale.

In Fig. 2 I have attempted to illustrate the structural nature of the working surface 5 of a contact formed in accordance with my invention. The main body portion of the contact point consists of highly refractory material A, illustrated as very finely divided, as tungsten in the crystalline form, 10 and the working surface is formed of a layer of more fusible material B, as of platinum, applied thereto and fused into the interstices between the tungsten particles in the above described manner, the tungsten particles having been previously closely compacted together under great pressure. This 15 results in a composite contact point having a main body portion A of finely divided closely compacted particles and a working 20 surface B of another material in the non-divided state, the latter material flowing into and completely filling the interstices between the finely divided particles near the 25 surface of the main body portion. For convenience in illustration I have shown the more fusible metal B as only penetrating the main body to a comparatively short depth below the surface although in practice the impregnation probably goes much deeper.

30 In fact, by properly proportioning the size and porosity of the absorbing particles or by continuing the sweating operation long enough the main body may become impregnated throughout. In all cases the impregnation 35 is more complete near the surface than deeper down, and the composition of the contact varies in a graded manner from the surface inwardly, the variation taking place progressively from the layer B to the 40 extent of the impregnation.

Having thus described my invention, what I claim is:—

1. The process of producing metallic bodies which consists of molding a finely 45 disintegrated metallic constituent of high melting point to the desired form, applying a layer of a constituent of lower melting point to the surface of the body and subjecting the composite body thus formed to 50 a temperature sufficient to melt the constituent of the lower melting point.

2. The process of producing metallic

bodies which consists of molding and compacting a finely disintegrated metallic constituent of high melting point to the desired 5 form under pressure, applying a layer of a constituent of lower melting point to the surface of the body, and subjecting the composite body thus formed to a temperature sufficient to melt the less refractory constituent 6 under non-oxidizing atmospheric conditions.

3. The process of producing composite metallic bodies which consists of molding and compacting a finely divided metallic 65 element of a high melting point into the desired form under great pressure, applying a layer of a less refractory element to the body, and sweating the less refractory element into the more refractory element by 70 subjecting, under non-oxidizing conditions, the composite body to a temperature intermediate the melting points of the constituent elements.

4. The process of producing composite 75 tungsten bodies, which consists of molding and compacting finely divided tungsten into the desired form under great pressure, applying a layer of an element of lower melting point than that of tungsten to the surface of the body thus formed, and sweating the less refractory element into the tungsten body by subjecting the composite body 80 in a neutral atmosphere to a temperature sufficiently high to melt the less refractory 85 element but lower than the melting point of tungsten.

5. The process of producing composite tungsten and platinum bodies which consists 90 in molding and compacting finely divided tungsten to the desired form under great pressure, applying a coating of platinum to the body thus formed, and sweating the platinum into the tungsten by subjecting the composite body in a neutral atmosphere 95 to a temperature intermediate the melting points of tungsten and platinum.

In testimony whereof, I hereunto affix my signature in the presence of two witnesses.

CHARLES L. GEBAUER.

Witnesses:

LUCIE C. EHRKE,  
H. B. MCGILL.